

## UNITED STATES PATENT OFFICE

HERMANN BERTHOLD AND PAUL RABE, OF LEVERKUSEN-ON-THE-RHINE, GERMANY,  
ASSIGNORS TO GENERAL ANILINE WORKS, INC., OF NEW YORK, N. Y., A CORPORATION OF DELAWARE

## PROCESS OF DYEING ACETATE SILK

No Drawing. Application filed June 30, 1928, Serial No. 289,614, and in Germany July 11, 1927.

The present invention relates to improvements in dyeing cellulose acetates with water-soluble dyestuffs having affinity for cellulose acetates and to products suitable for carrying out said process.

In accordance with the present invention, in dyeing cellulose acetates, such as acetate silk, acetate films and the like, a hydrogenated carbocyclic base having a benzene or 10 naphthalene nucleus, the nitrogen atom being attached to a carbon atom in said nucleus is added to the dyeing bath. This addition facilitates the dyeing of the acetyl cellulose without the harmful secondary effects generally caused by other alkaline reacting agents, i. e. partial saponification accompanied by deterioration of the mechanical strength and the luster of the acetyl cellulose products. Moreover, it is possible according to the present process to dye acetate silk particularly clear shades by means of many wool dyestuffs, especially such as contain sulfur groups, which until now could only be applied to cellulose acetate fibers with 25 difficulty.

Such bases are, for instance, hexahydroaniline and substitution products thereof, for example, hexahydro-methylaniline, hexahydro-ethylaniline, also the homologues of hexahydro-aniline, for example, hexahydro-toluidines, such as hexahydroethyl-ortho-toluidine and hexahydro-ortho- (and meta-) toluidine, hexahydroxytoluidines, such as hexahydro-meta-xylidine and finally the hydrogenated naphthalenediamines, for example, hydrogenated 1:5- and 1:7-naphthalenediamines.

The quantity of the bases added to the dyeing bath may be varied within wide limits. 40 We prefer to use about 1 to 3 per cent calculated on the amount of the bath. The dyeing is effected in the usual manner, for example, by dissolving the dyestuff in water, adding the base, introducing the material to be dyed 45 while heating to about 50-75° C., dyeing at this temperature for one-half to one hour, rinsing and drying.

In case a dyestuff containing an acid group is used, a salt of said dyestuff with a hydrogenated aromatic base can be isolated and

used in the dyeing process in the customary manner, instead of adding the said base to the dyeing bath. Such salts can be prepared, for example, by dissolving the sodium salt of the dyestuff in alcohol, adding hydrochloric acid, whereby the so-called "anhydroform" of the sulfonic acid separates, which latter can be transformed into the salt to be prepared by simple rubbing with the respective base.

The following examples will illustrate our invention, without limiting it thereto:

*Example 1.*—0.1 gram of the sodium salt of 1-amino-4-hexahydroanilido anthraquinone-2-sulfonic acid is dissolved in 100 cc. of water. About 1 gram of hexahydroaniline is added and the wetted goods are introduced into the solution at 60-70° C. and dyed at 65-75° C. for about one hour, rinsed and dried. The acetate silk is dyed in clear blue shades. When applying in this example instead of the free dyestuff its salt with hexahydroaniline, the same result is obtained without the addition of free hexahydroaniline.

*Example 2.*—Orange II (see Color Index 1924, No. 151) is used for dyeing in the same manner, when deeper shades are obtained compared with those resulting from the customary dyeing methods without the addition of the above bases.

*Example 3.*—Benzo brown G (see Color Index 1924, No. 331) with the addition of 3% of hexahydroaniline dyes acetate silk better and in clearer shades than according to the dyeing methods hitherto known.

*Example 4.*—2% of rhodulin orange NO (see Color Index, 1924, No. 778) with the addition of 3% of hexahydroaniline dyes acetate silk considerably better than according to the dyeing methods hitherto known.

Other water-soluble dyestuffs can be used, for example, brilliant rhodulin violet R (see German Patent 81,963), methyleneblue BB (see Color Index 1924, No. 922), safranine FF extra No. 0 (see Color Index 1924, No. 841), and the like.

We claim:

1. Process which comprises dyeing cellulose acetate with a dyeing bath containing a

55

60

65

70

75

80

85

90

95

100

water-soluble dyestuff having affinity for cellulose acetate fibres and a hydrogenated carbocyclic base having a benzene or naphthalene nucleus, the nitrogen atom being attached to a carbon atom in said nucleus.

2. Process which comprises dyeing cellulose acetate with a dyeing bath containing a water-soluble dyestuff having affinity for cellulose acetate fibres and hexahydroaniline.

10 3. Process which comprises dyeing acetate silk with a dyeing bath containing 1-amino-4-hexahydro-anilido - anthraquinone - 2 - sulfonic acid and hexahydroaniline.

4. A dyeing composition comprising a water-soluble dyestuff having affinity for cellulose acetate fibres and a hydrogenated carbocyclic base having a benzene or naphthalene nucleus, the nitrogen atom being attached to a carbon atom in said nucleus.

20 5. A dyeing composition comprising a water-soluble dyestuff having affinity for cellulose acetate fibres and hexahydroaniline.

6. A dyeing composition comprising 1-amino-4-hexahydroanilido-anthraquinone-2-sulfonic acid and hexahydroaniline.

7. A dyeing bath containing a water-soluble dyestuff having affinity for cellulose acetate fibres and a hydrogenated carbocyclic base having a benzene or naphthalene nucleus, the nitrogen atom being attached to a carbon atom in said nucleus.

30 8. As a new article of manufacture, cellulose acetate dyed with a water-soluble dye stuff having affinity for cellulose acetate fibres in the presence of a hydrogenated carbocyclic base having a benzene or naphthalene nucleus, the nitrogen atom being attached to a carbon atom in said nucleus.

40 9. As a new article of manufacture, acetate silk dyed with a water-soluble dyestuff having affinity for acetate silk in the presence of hexahydroaniline.

10. As a new article of manufacture, acetate silk dyed in clear blue shades with 1-amino-4-hexahydroanilido-anthraquinone-2-sulfonic acid in the presence of hexahydroaniline.

In testimony whereof we have hereunto set our hands.

60 HERMANN BERTHOLD. [L. S.]  
PAUL RABE. [L. S.]